

[54] CONTAINER CAP HAVING A PEELABLE LINER

[56]

## References Cited

## U.S. PATENT DOCUMENTS

|           |        |                                |
|-----------|--------|--------------------------------|
| 2,567,067 | 9/1951 | Grupp et al.                   |
| 3,312,005 | 4/1967 | McElroy                        |
| 3,361,281 | 1/1969 | Kehe                           |
| 3,557,987 | 1/1971 | Singer, Jr.                    |
| 3,633,781 | 1/1972 | Zapata                         |
| 4,111,323 | 9/1978 | Ichinose et al. .... 215/347 X |

## FOREIGN PATENT DOCUMENTS

2178313 9/1978 France

Primary Examiner—Donald F. Norton  
Attorney, Agent, or Firm—Pennie & Edmonds

[57]

## ABSTRACT

A container cap having a coated metal shell. A peelable adhesive layer joins a liner to the shell. The peelable adhesive layer comprises a local coating resin layer having a diameter less than that of the metal shell and a layer of an epoxy resin.

10 Claims, 3 Drawing Figures

[75] Inventors: Go Kunimoto, Fujisawa; Isao Ichinose, Hiratsuka; Noboru Suzuki, Fujisawa; Fumio Mori, Yokohama, all of Japan

[73] Assignee: Toyo Seikan Kaisha Ltd., Tokyo, Japan

[21] Appl. No.: 90,627

[22] Filed: Nov. 2, 1979

## [30] Foreign Application Priority Data

Nov. 2, 1978 [JP] Japan 53-150373[U]

[51] Int. Cl.<sup>3</sup> B65D 53/00  
[52] U.S. Cl. 215/228; 215/230; 215/347

[58] Field of Search 215/228, 230, 341, 347, 215/343



FIG. 1



FIG. 2



FIG. 3



## CONTAINER CAP HAVING A PEELABLE LINER

## TECHNICAL FIELD

The present invention relates to a container cap having a peelable liner. More particularly, the invention relates to a container cap having an easily peelable liner and an interface layer joining the liner to a coated metal shell where the interface layer resists breaking up into small pieces and so forming objectionable dust particles during cap forming procedures.

## BACKGROUND ART

Container caps in the form of crown caps or caps for wide mouth vessels have been formed in the past by coating a surface-protecting paint on a metal sheet, forming the coated metal sheet into a crown shell or cap shell and then bonding a liner or packing material to the interface of the formed shell.

In premium sales of bottled drinks and the like, there is often adopted a system in which a purchaser returns a predetermined number of liners or a liner having a win mark printed thereon in return for which a prize is sent to the purchaser. In crown shells or caps for use in such premium sales, it is important that a liner or packing should be easily peelable from the crown shell or cap. Furthermore, from the sanitary viewpoint, it is important that any printed surface of a liner be out of direct contact with the packed drink. Since a liner per se is usually applied to the interface of a crown shell or cap shell in a melted state, it is preferred that when a liner is peeled from a cap, that any ink layer applied to the crown shell or cap shall be transferred to the peeled liner.

In order to provide caps meeting the above requirements, usually a plurality of coating layers are formed on a metal sheet constituting a cap shell and peeling is effected in the interface between two coated layers. However, coating layers forming the easily peelable interface are readily broken into small pieces during the steps of press or draw forming of a metal sheet into a crown shell or cap shell, during transport of the crown or cap shells, during capping and so-called roll-on processing, all of which results in objectionable dust particles being formed. This phenomenon is not preferred from a sanitary viewpoint and it reduces the commercial value of products.

It is therefore an object of our invention to provide for a cap having an easily peelable liner and which will not form objectionable dust particles during processing steps.

## DISCLOSURE OF INVENTION

Broadly a cap constructed according to our invention utilizes a peelable interface that is formed between a layer of a hydrocarbon resin or natural resin and a layer containing an epoxy resin. These two layers are applied on the inner facing surface of a coated metal sheet such that the hydrocarbon resin or natural resin layer has a local or limited area having a diameter less than that of the shell to be formed or of the liner to be fitted into the shell. By this means, a liner affixed to the layer containing the epoxy resin will have excellent peelability properties with respect to the epoxy layer and the layer forming the peelable interface will have excellent dust-resisting properties.

More specifically, in accordance with the present invention, there is provided a container cap having a

peelable liner, which comprises a shell formed of a coated metal plate and a thermoplastic resin liner applied to the inner facing surface of the shell. The liner is bonded to the shell by way of a peelable adhesive interface between a layer composed of a hydrocarbon resin or natural resin which is applied locally to a limited area of the inner face of the shell so as to have a diameter less than that of the shell or the liner and a diameter greater than the peelable area of the liner. A layer containing an epoxy resin which is formed on the hydrocarbon resin or natural resin layer surrounds and overlies the layer of hydrocarbon or natural resins.

## BRIEF DESCRIPTION OF THE DRAWINGS

FIG. 1 is an enlarged sectional view illustrating a coated metal sheet prior to being formed into a crown or cap shell;

FIG. 2 is a sectional view illustrating a container cap constructed according to the invention in the form of a crown cap; and

FIG. 3 is a sectional view illustrating a container cap constructed according to the invention in the form of a pilfer-proof cap.

## BEST MODE FOR CARRYING OUT THE INVENTION

Referring to FIG. 1 there is illustrated the sectional structure of a coated metal sheet prior to being formed into a cap shell. Layers 2 of a known protecting paint are applied to both the surfaces of a metal substrate 1 which may comprise a tin-deposited steel plate or a tin-free steel plate (steel plate electrolytically treated with chromic acid). A peelable adhesive layer 3 of a hydrocarbon resin or natural resin is locally applied to the surface of the coated metal sheet to which a liner is to be applied. The shape and size of the layer 3 is limited so that the layer 3 has a diameter greater than that of the peelable portion of the liner to be applied and less than that of the metal shell.

A coating layer 4 containing an epoxy resin is applied on the entire surface of the layer 3 and a printing ink layer 5 having prize marks or indicia is formed on the layer 4 at a position corresponding to the local coating layer 3. An adhesive paint layer 6 is applied on the printing ink layer 5.

Referring to FIG. 2 a crown cap is illustrated formed from the above-mentioned coated metal sheet which has been punched and formed into a circular top portion 7 and a corrugated skirt 8. In the present invention, the local coating layer 3 composed of a hydrocarbon resin or natural resin is located on the inner side of the metal shell and has a diameter less than that of the top portion 7. This feature is very important in preventing formation of dust particles during processing operations.

A liner 9 of a synthetic resin is applied to the inner side of the top portion 7 of the crown shell and this liner 9 is bonded to the shell through an adhesive paint layer 6. The liner 9 may have a thick portion 10 providing good sealing of the liner 9 to the mouth of a container (not shown).

An important feature of the present invention resides in that the layer 3 composed of a hydrocarbon resin or natural resin forms an adhesive interface with the layer 4 comprising an epoxy resin to give a much better peelability characteristic than interfaces of known layer combinations. A further feature is that the combined portion of the resin layers 3 and 4 are locally applied on the

inner side of the shell such that the diameter of the combined portion of the layers is less than that of the top portion 7 and greater than that of the liner 9. This prevents formation of dust particles during the steps of formation of the cap shell and during transportation, sealing and opening of the container cap.

In the instant specification and appended claims, the term "easily peelable adhesive interface" is defined as an interface between two layers which are bonded together to such an extent that they will not peel from each other during ordinary handling but may be easily peeled from each other by finger pressure. Ordinarily, this easily peelable adhesive interface has a peel strength in the range of 20 to 600 g/cm. In the present invention a layer 3 of a hydrocarbon resin or natural resin and an epoxy resin layer 4 will form such an easily peelable adhesive interface.

As pointed out hereinbefore, in conventional combined resin layers forming peelable adhesive interfaces, dust particles are formed in large quantities during processing and handling of the container caps. In the present invention, the combined resin layers 3 and 4 are formed on the inner side of the shell such that the diameter of the combined portions of the layers is less than that of the shell and greater than that of the liner to be applied such that the underside of the liner forms a peelable portion of the liner. That is, the combined resin layers 3 and 4 are located in the top portion of the shell which is not bent, or only slightly bent, during forming of a cap shell. Accordingly, formation of dust particles can be prevented during press forming or draw forming of the metal sheet. Furthermore, the portion where the combined resin layers 3 and 4 are located is protected by the skirt 8 thus preventing breaking of the interface area and subsequent dust formation during handling and transportation of the cap prior to being applied to a container. This interface area is protected during seal-

5 indene resins, terpene resins, rosin resins, rosin esters and modified rosin resins are especially preferred.

As petroleum resins, known products are obtained by heat-polymerizing a petroleum type unsaturated hydrocarbon such as cyclopentadiene or a higher olefinic hydrocarbon having 5 to 11 carbon atoms in the presence of a catalyst. In the present invention, any of these known petroleum resins may be used for formation of the coating layer 3. As the coumarone-indene resin, there are known resins having a relatively low degree of polymerization, which are obtained by polymerizing a tar fraction composed mainly of coumarone and indene (ordinarily boiling at 160° to 180° C.) in the presence of a catalyst or under application of heat. Any of these known resins can be used in the present invention. As the terpene resin, there can be used synthetic and natural polymers of terpene type hydrocarbons, particularly resins obtained by polymerizing a terpene oil or nopinene fraction in the presence of a catalyst. As the rosin, there can be used so-called raw rosins such as gum rosin and wood rosin, rosin esters obtained by esterifying abietic acid in the rosin, such as rosin glycerin ester (ester gum), diethylene glycol diabietate, diethylene glycol 2-hydroxyabietate, rosin monoethylene glycol ester and rosin pentaerythritol ester. These rosins may be modified with known thermosetting resins or the like.

20 As the epoxy resin constituting the layer 4, there are employed polymeric compounds having at least two epoxy compounds in the molecule, precondensates thereof and their combinations with low-molecular-weight or high-molecular-weight curing agent compounds having a reactivity with epoxy groups.

25 Ordinarily, an epoxy resin formed by condensing epichlorohydrine with a polyhydric phenol is preferably employed. An epoxy resin of this type has a molecular structure represented by the following formula:



30 ing of a cap to a container by the liner 9 thus further reducing probability of formation of dust particles. A hydrocarbon resin or natural resin has a viscosity suitable for lithographic printing, relief printing, intaglio printing and screen printing. Accordingly an advantage of using these materials is that local coating to form the interface area can be accomplished very easily by printing.

35 When the liner 9 is peeled from a cap constructed according to the invention, the peripheral portion of the liner 9 is pressed by a nail or tool whereby peeling is initiated between the local coating layer 3 and the epoxy resin layer 4. This results in breakage occurring between the coating layer 4 and the layer 6 at the peripheral portion of the liner. Then, peeling is easily advanced in the interface between the layers 3 and 4. The liner 9 is thus easily peeled from the top portion 7 of the shell in a state where the printing ink layer 5 will be transferred to the liner 9 with the portions of the layers 4 and 6 located radially inwardly of the liner remaining attached to the liner.

40 The resin constituting the local coating layer 3 should have a softening point (as measured according to the ring and ball method) lower than 180° C., and preferably lower than 120° C., in view of the adaptability to printing operations. Petroleum resins, coumarone-

45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920

hydride, cyclopentadiene-methyl maleate adduct, dodecylsuccinic anhydride, dichloromaleic anhydride and chlorendic anhydride.

The curing agent is used in an amount of 2 to 150 parts by weight, preferably 20 to 60 parts by weight, per 100 parts by weight of the epoxy resin component (all "parts" and "%" given hereinafter are by weight unless otherwise indicated).

In accordance with one preferred embodiment of the present invention, a mixture of an epoxy resin component as mentioned above and at least one thermosetting resin selected from the group consisting of resol type phenol-formaldehyde resins, urea-formaldehyde resins and melamine-formaldehyde resins is used for formation of the layer 4. The mixing ratio of the two resin components can be changed in a broad range. Ordinarily, it is preferred that the mixing ratio of the epoxy resin to the thermosetting resin be in the range of from 5/95 to 95/5, especially 40/60 to 90/10. The epoxy resin and thermosetting resin may be used in the form of a blend for 20 formation of the coating layer 4 or they may be used after they have been precondensed.

In view of processability and corrosion resistance, a vinyl resin is preferred for formation of the protecting layer 2. As the vinyl resin, a copolymer of (a) vinyl chloride is mixed with (b) at least one ethylenically unsaturated monomer selected from vinyl acetate, vinyl alcohol, vinyl acetal, acrylic acid, methacrylic acid, maleic acid, fumaric, itaconic acid, alkyl acrylates, alkyl methacrylates and vinylidene chloride. The mixing 30 ratio of vinyl chloride (a) to other ethylenically unsaturated monomer (b) may be changed in a broad range. Ordinarily, however, it is preferred that the mixing molar ratio (a)/(b) be in the range of from 95/5 to 60/40, particularly from 90/10 to 70/30. The molecular weight of the vinyl resin is not particularly critical provided that the vinyl resin has a film-forming molecular weight. As preferred examples of the vinyl resin, there can be mentioned a vinyl chloride-vinyl acetate copolymer, a partially saponified vinyl chloride-vinyl acetate copolymer, a partially saponified and partially acetalized vinyl chloride-vinyl acetate copolymer, a vinyl chloride-vinyl acetate-maleic anhydride copolymer and a vinyl chloride-vinylidene chloride-acrylic acid copolymer.

Furthermore, an epoxy resin, an amino resin, a phenolic resin, an acrylic resin and a vinyl butyral resin may be used singly or in the form of a mixture of two or more of them. These resins may be used in combination with the above-mentioned vinyl resins.

A synthetic resin having appropriate cushioning and sealing properties, for example, an olefin resin such as polyethylene, an ethylene-vinyl acetate copolymer or an ethylene-propylene copolymer or a soft vinyl chloride resin, is used as the liner 9. As the adhesive paint layer 6, an acid-modified olefin resin or oxidized polyethylene is used for an olefin type resin liner, and a vinyl resin paint such as mentioned above or an acrylic resin paint is used for a vinyl chloride resin liner.

For formation of the liner 9, in view of the adaptability to the forming operation, there is preferably adopted a method in which a thermoplastic resin is extruded in a cap shell and shaping of a liner and heat bonding are simultaneously performed by mold pressing, or a method in which a flowable composition such as a plasti-sol is supplied into a shell and the composition is spread by a centrifugal force to form a liner. Furthermore, there may be adopted a method in which a disc

liner is formed outside a shell and it is bonded to the top portion of the shell.

The container cap of the present invention may be formed in a so-called liner-provided cap. In this embodiment, as shown in FIG. 3, the liner 9' comprises a thick sealing portion 10' and a thin central portion 11' and a completely cut line or breakable weakened line 12' is formed in the boundary between the two portions 10' and 11' so that only the central portion 11' of the liner 9' forms a peelable portion which is peeled off. Accordingly, even after peeling of the liner, the cap still retains the sealing property.

The local coating layer 3' of a hydrocarbon resin or natural resin may be formed so that it covers the entire 15 surface of the liner or, it may be formed only on the central portion of the liner.

The structure and effect of the present invention will now be described with reference to the following Examples.

#### EXAMPLE 1

A 30% solution of a vinyl chloride-vinyl acetate copolymer (VMCH® manufactured by UCC) in a mixed solvent containing equal amounts of methyl cellosolve and methyl-ethyl ketone was roll-coated as an undercoat paint on both the surfaces of an aluminum plate having a thickness of 0.25 mm so that the dry thickness of the coating was 6μ, and the coating was heated and baked at 190° C. for 10 minutes.

A circular trademark having an outer diameter of 70 mm was printed on one surface of the surface-coated plate by using an ordinary metal printing ink. Then, an epoxy ester type paint was coated in a thickness of 5μ on the printed surface and the coating was dried.

On the other surface of the coated plate, a circular print layer having an outer diameter of 26 mm and a thickness of 3μ was formed with a mineral spirit solution (solid content = 75%) of a hydrocarbon resin (Hi-Lez P-100 manufactured by Mitsui Petrochemical) by 35 using a printing machine so that the center of the print layer was in agreement with the center of the above-mentioned printed trademark, and the print layer was heated and dried at 180° C. for 10' minutes. Then, an epoxy-amino resin paint (a 30% solution of 90 parts of 40 Epikote® #1009 manufactured by Shell and 10 parts of Beccamine® 138 manufactured by Nippon Reichhold mixed in equal amounts of Solvesso #100 and methyl-ethyl ketone) was roll-coated in a thickness of 2μ on the hydrocarbon resin-printed surface and baked and cured 45 at 190° C. for 10 minutes.

A prize mark was printed on the epoxy-amino resin coating layer in a circular area having an outer diameter of about 26 mm by using an ordinary metal ink so that the prize mark was located at the same position as that of the lower hydrocarbon resin layer, and the printed part was cured. Finally, an epoxy paint containing 20% of oxidized polyethylene (a xylene solution of a mixture formed by incorporating oxidized polyethylene having a density of 0.98 and a softening point of 132° C. into a 55 90/10 blend of Epikote #1007/phenol-formaldehyde resin) was coated in a thickness of 5μ entirely on the prize mark-printed surface and heated and cured at 190° C. for 10 minutes. Thus, a coated aluminum plate having printed areas on both the surfaces was prepared. The coated plate was punched into a cylinder so that the prize mark-printed surface was located inside and the centers of the printed areas were in agreement with the center of the resulting cap and a perforation cut line 60 65

was formed. Thus, a roll-on pilfer-proof cap shell having an inner diameter of 38 mm and a height of 17 mm was prepared.

Molten low density polyethylene having a melt index of 7 was supplied on the inner face of the cap shell in an amount of 0.6 g per cap and punched by cooled press-forming punch to form a cap shell having a polyethylene liner in the shape as shown in FIG. 3. The outer diameter of the cap shell was 36 mm and the diameter of the portion to be peeled was 25 mm.

The cap was tested with respect to processability (formation of dusts at the cap forming step and the punching step), liner bonding property (falling or sticking of the liner at the hoppering test) and liner peelability (peelability of the liner from the cap after it was separated from a glass bottle to which the cap had been sealed). Obtained results are shown in Table 1.

#### COMPARATIVE EXAMPLE 1

A coated plate was prepared in the same manner as 20 described in Example 1 except that the hydrocarbon resin was printed on the entire surface of the plate, and a cap shell was prepared from this coated plate in the same manner as described in Example 1. The cap was tested with respect to the items described in Example 1. 25 Obtained results are shown in Table 1.

#### COMPARATIVE EXAMPLE 2

A coated aluminum plate was prepared in the same manner as described in Example 1 except that the hydrocarbon resin was not printed on the plate. A cap shell was formed from this coated plate in the same manner as described in example 1 and was tested in the same manner as in Example 1 to obtain results shown in Table 1.

#### COMPARATIVE EXAMPLE 3

A coated aluminum plate was formed in the same manner as described in Example 1 except that polyethylene wax was used instead of the hydrocarbon resin 40 used in Example 1. A cap shell was prepared from this coated plate in the same manner as described in Example 1 and tested in the same manner as in Example 1 to obtain results shown in Table 1.

#### EXAMPLE 2

A base coat layer (epoxy-amino resin paint), a trademark print and an overcoat layer (epoxy ester paint) were formed on one surface (the outer face of the resulting crown) of a surface-treated steel plate having a 50 thickness of 0.25 mm (Hi-Top®) manufactured by Toyo Kohan), and an anti-corrosive lacquer comprising 70 parts of a vinyl chloride-vinyl acetate copolymer, 25 parts of a bisphenol type epoxy resin and 5 parts of an

amino resin (butylated urea resin) in an organic solvent was roll-coated on the other surface (inner face of the resulting crown) so that the thickness after drying and curing was 3μ. The plate was then heated at 190°C. for 10 minutes. A kerosine solution (solid content = 40%) of a natural resin (rosin) was coated on the anti-corrosive lacquer layer in a thickness of 5μ (1) on the entire surface of the anti-corrosive lacquer layer, (2) on a circular area having an inner diameter of 26 mm or (3) on a circular area having an inner diameter of 28 mm and heated and dried at 180°C. for 10 minutes.

An epoxy-phenolic paint (a 33% solution of a 90/10 blend of Epikote #1009/resol type phenolic resin in a mixed solvent of xylene and isobutyl ketone) was roll-coated on the entire surface of the so-formed natural resin layer so that the thickness after drying was 3μ and heated at 190°C. for 10 minutes to form a coating layer.

A prize mark was printed on the so-formed epoxy-phenolic resin layer only in the area where the natural resin layer was present below by using an ordinary metal printing ink of the alkyd resin type and the printed prize mark was dried. A mixture formed by incorporating 20% of oxidized polyethylene having a density of 1.0 and a softening point of 135°C. into the above-mentioned epoxy-phenolic resin paint was coated as an adhesive entirely on the inner face (thickness = 6μ) and heated at 190°C. for 10 minutes to form a coated plate having printed areas on both the surfaces.

The printed coated plate was formed into a crown shell having an inner diameter of 26 mm by crown forming press so that the prize mark-printed surface was located inside and the center of the circular natural resin coating layer having an inner diameter of 26 or 28 mm was in agreement with the center of the top portion of the crown shell.

A molten mass of low density polyethylene having a melt index of 7 and a density of 0.92 was supplied to the inner face of the crown shell in an amount of 0.25 g per shell, and punched by a cooled forming punch to form a crown shell having a polyethylene liner having an outer diameter of 26 mm.

The crown shell was tested with respect to processability (formation of dusts at the pressing, punching and capping steps), liner bonding property (falling or sticking of the liner on hoppering at the capping step) and liner peelability (peelability of the liner from the opened crown which had been sealed to a bottle). The results obtained are shown in Table 2.

For comparison, a crown shell was prepared in the same manner as described above except that the natural resin layer was not formed at all, and the crown shell was similarly tested. Obtained results are shown in Table 2.

TABLE 1

| Sample                | Amount (mg) of Formed Dusts <sup>1)</sup><br>cap forming | Amount (mg) of Formed Dusts <sup>1)</sup><br>punching | Liner Bonding Property | Liner Peeling Ability <sup>2)</sup> (g/cm) | Re-sealing Property <sup>3)</sup> | Remarks                                                     |
|-----------------------|----------------------------------------------------------|-------------------------------------------------------|------------------------|--------------------------------------------|-----------------------------------|-------------------------------------------------------------|
| Example 1             | 1                                                        | 0                                                     |                        | 450                                        |                                   | prize mark was transferred to liner entire liner was peeled |
| Comparative Example 1 | 150                                                      | 102                                                   | Δ- X                   | 300                                        | X                                 |                                                             |
| Comparative Example 2 | 3                                                        | 0                                                     |                        | not peelable <sup>4)</sup>                 | —                                 |                                                             |
| Comparative Example 3 | 85                                                       | 73                                                    | X                      | measurement                                | X                                 | liner often dropped                                         |

TABLE 1-continued

| Sample | Amount (mg) of<br>Formed Dusts <sup>1)</sup> | Liner<br>cap<br>forming | Liner<br>punching | Bonding<br>Property | Liner<br>Peela-<br>bility <sup>2)</sup><br>(g/cm) | Re-sealing<br>Property <sup>3)</sup> | Remarks |
|--------|----------------------------------------------|-------------------------|-------------------|---------------------|---------------------------------------------------|--------------------------------------|---------|
|        |                                              |                         |                   |                     | impossible <sup>5)</sup>                          |                                      |         |

## Note

<sup>1)</sup> Amount (mg) of dusts (pieces of coatings) formed in 100 caps at each step<sup>2)</sup> Peel strength (g/cm) of liner from cap<sup>3)</sup> Sealing property of cap after peeling of liner<sup>4)</sup> Liner could not be peeled because of too strong bonding<sup>5)</sup> liner was peeled before measurement because of too weak bonding

: good

Δ: ordinary

X: bad

TABLE 2

| Crown Shell                                             | Amount (g) of<br>Dust Formed |    | Liner<br>Bonding<br>Property | Liner<br>Peelability<br>(g/cm) | Remarks                                   |
|---------------------------------------------------------|------------------------------|----|------------------------------|--------------------------------|-------------------------------------------|
| natural resin<br>layer 26 mm in<br>diameter             | 1                            | 0  |                              | 430                            | prize mark was<br>transferred to<br>liner |
| natural resin<br>layer 28 mm in<br>diameter             | 36                           | 27 | Δ                            | 270                            | prize mark was<br>transferred to<br>liner |
| natural resin<br>layer coated<br>on entire sur-<br>face | 102                          | 89 | X                            | 250                            | prize mark was<br>transferred to<br>liner |
| natural resin<br>layer not<br>coated                    | 2                            | 0  |                              | not peelable                   |                                           |

## We claim:

1. A container cap comprising a metal shell, a thermoplastic resin peelable liner on the inside of said shell, a peelable adhesive layer having a diameter less than that of said metal shell and larger than that of a peelable portion of the liner, and an epoxy resin coating layer secured to said liner overlying the inside surface of said metal shell and said peelable adhesive layer to form an easily peelable adhesive interface with said peelable adhesive layer whereby pressing the periphery of the liner overlying said inner face will cause a break in the epoxy resin layer to allow easy peeling of the liner from the shell at the interface.

2. A container cap according to claim 1 wherein said peelable adhesive layer has a softening point below 180° C.

3. A container cap according to claim 1 wherein said peelable adhesive layer comprises a hydrocarbon resin.

4. A container cap according to claim 3 wherein said hydrocarbon resin comprises a petroleum resin.

5. A container cap according to claim 3 wherein said hydrocarbon resin layer comprises a coumarone-indene resin.

6. A container cap according to claim 1 wherein said peelable adhesive layer comprises a natural resin.

7. A container cap according to claim 6 wherein said natural resin comprises a rosin.

8. A container cap according to claim 6 wherein said natural resin comprises a rosin ester.

9. A container cap according to claim 6 wherein said natural resin comprises a terpene resin.

10. A container cap according to claim 1 wherein said peelable adhesive layer is formed by printing.

\* \* \* \* \*

UNITED STATES PATENT AND TRADEMARK OFFICE  
CERTIFICATE OF CORRECTION

PATENT NO. : 4,310,100

Page 1 of 2

DATED : January 12, 1982

INVENTOR(S) : Go Kunimoto et al

It is certified that error appears in the above-identified patent and that said Letters Patent is hereby corrected as shown below:

Columns 8 and 9, Tables 1 and 2 should appear as follows:

TABLE I

| Sample                | Amount (mg) of Formed Dusts <sup>1)</sup> |     | Liner Bonding Property | Liner Peelability <sup>2)</sup> (g/cm) | Re-sealing Property <sup>3)</sup> | Remarks                             |
|-----------------------|-------------------------------------------|-----|------------------------|----------------------------------------|-----------------------------------|-------------------------------------|
| Example 1             | 1                                         | 0   | O                      | 450                                    | O                                 | prize mark was transferred to liner |
| Comparative Example 1 | 150                                       | 102 | A-X                    | 300                                    | X                                 | entire liner was peeled             |
| Comparative Example 2 | 3                                         | 0   | O                      | not peelable <sup>4)</sup>             | --                                |                                     |
| Comparative Example 3 | 85                                        | 73  | X                      | measurement                            | X                                 | liner often dropped                 |

TABLE I-continued

| Sample                   | Amount (mg) of Formed Dusts <sup>1)</sup> |  | Liner Bonding Property | Liner Peelability <sup>2)</sup> (g/cm) | Re-sealing Property <sup>3)</sup> | Remarks |
|--------------------------|-------------------------------------------|--|------------------------|----------------------------------------|-----------------------------------|---------|
| impossible <sup>5)</sup> |                                           |  |                        |                                        |                                   |         |

Note

1) Amount (mg) of dusts (pieces of coatings) formed in 100 caps at each step

2) Peel strength (g/cm) of liner from cap

3) Sealing property of cap after peeling of liner

4) Liner could not be peeled because of too strong bonding

5) Liner was peeled before measurement because of too weak bonding

O good

A ordinary

X bad

UNITED STATES PATENT AND TRADEMARK OFFICE  
CERTIFICATE OF CORRECTION

PATENT NO. : 4,310,100

Page 2 of 2

DATED : January 12, 1982

INVENTOR(S) : Go Kunimoto et al

It is certified that error appears in the above-identified patent and that said Letters Patent is hereby corrected as shown below:

TABLE 2

| Crown Shell                                             | Amount (g) of<br>Dust Formed |         | Liner<br>Bonding<br>Property | (g/cm)       | Liner<br>Peelability                      | Remarks |
|---------------------------------------------------------|------------------------------|---------|------------------------------|--------------|-------------------------------------------|---------|
|                                                         | pressing                     | capping |                              |              |                                           |         |
| natural resin<br>layer 26 mm in<br>diameter             | 1                            | 0       | ○                            | 430          | prize mark was<br>transferred to<br>liner |         |
| natural resin<br>layer 28 mm in<br>diameter             | 36                           | 27      | △                            | 270          | prize mark was<br>transferred to<br>liner |         |
| natural resin<br>layer coated<br>on entire sur-<br>face | 102                          | 89      | ×                            | 250          | prize mark was<br>transferred to<br>liner |         |
| natural resin<br>layer not<br>coated                    | 2                            | 0       | ○                            | not peelable |                                           |         |

Signed and Sealed this  
Twentieth Day of April 1982

(SEAL)

Attest:

GERALD J. MOSSINGHOFF

Attesting Officer

Commissioner of Patents and Trademarks